

M. M. MERRITT,  
GALVANOPLASTIC PROCESS AND PRODUCT,  
APPLICATION FILED DEC. 8, 1917.

1,282,269.

Patented Oct. 22, 1918.



Testimony:  
Merritt, M. Merritt,  
by Emery Booth, James Varney,  
Hedges.

# UNITED STATES PATENT OFFICE.

MATTHEW M. MERRITT, OF SOUTH MIDDLETON, MASSACHUSETTS, ASSIGNOR TO COPPER PRODUCTS COMPANY, OF BOSTON, MASSACHUSETTS, A CORPORATION OF MAINE.

## GALVANOPLASTIC PROCESS AND PRODUCT.

1,282,269.

Specification of Letters Patent.

Patented Oct. 22, 1918.

Original application filed November 2, 1917, Serial No. 199,810. Divided and this application filed December 8, 1917. Serial No. 206,293.

To all whom it may concern:

Be it known that I, MATTHEW M. MERRITT, a citizen of the United States, and a resident of South Middleton, county of Essex, Commonwealth of Massachusetts, have invented an Improvement in Galvanoplastic Processes and Products "A," of which the following description, in connection with the accompanying drawings, is a specification, like characters on the drawings representing like parts.

This invention pertains to improvements in galvano plastic processes and products, but more particularly, though not exclusively, to the manufacture of articles such as manifolds for internal combustion engines such as aeroplane engines.

This application is a divisional of my co-pending application, Serial No. 199,810, filed

20 November 2, 1917.

In the drawings, which show one form of an illustrative embodiment of my invention:

Figure 1 shows a manifold; and

Fig. 2 is a diagrammatic section there-

25 through on the line 2—2 of Fig. 1.

Great difficulty has been experienced in constructing manifolds for aeroplane engines of the requisite light weight which are strong enough to withstand the constant and excessive vibrations occasioned by the operation of the engine. Such manifolds are very likely to develop cracks, particularly adjacent the bent portions thereof. It has heretofore been attempted to manufacture such manifolds by the electrolytic deposit of copper on cathodes of metal fusible at a low temperature, and on cathodes of wax painted with graphite or other electrically conductive material, the core being melted out after the electrolytic deposit. Manifolds made by the usual methods, above-described, have proved unsatisfactory because of brittleness and coarseness of texture of the deposited metal, this brittleness being accentuated at points adjacent curved portions of the deposit.

I have found that the deposits made as before described are rendered more uniform in quality by intermittent immersion of the cathode, as by attaching the same to a revolving wheel partially immersed in the electrolyte so that the entire cathode or a considerable portion thereof, preferably at least one-half, is only intermittently im-

mersed in the electrolyte. This aspect of my 55 invention is not claimed herein being comprised in the subject matter of a copending application Serial No. 247,966, filed August 2, 1918. While the intermittent immersion improves the texture of the deposited metal, 60 electrolytic deposits made on metallic cathodes having low melting points are, as heretofore made, likely to be rough and brittle. I believe this to be due to the tendency of certain ingredients of the fusible metal, 65 which is usually an alloy of lead, to be attacked by the electrolyte, and in some instances to be disassociated into negative ions traveling from the cathode to the anode.

Where, on the other hand, the cathode is 70 formed of non-conductive material removable by fusion, by a solvent, or otherwise, and the surface of which is coated with an electrically conductive paint, such as graphite, bronze powder and the like, the deposited copper, as heretofore practised, has been brittle and of slight tensile strength. 75 As stated in my co-pending application, filed herewith, I believe this to be due to the comparatively coarse texture of the conductive 80 coating which is necessarily full of interstices as compared with cast, rolled, or electrolytically deposited metal. The unevenness of attraction exerted by this surfacing of the cathode results in combining the deposited metal in relatively coarse crystalline 85 formation, which renders it brittle and of slight tensile strength.

I have found that the deleterious effects of a cathode composed of metal having a low 90 fusing-point may be minimized by coating the metal with a film of a foreign substance such as grease, and that if a layer of copper, preferably relatively thin, be electrolytically deposited subsequent to the application of the 95 grease and the surface of this metal treated with mercury or mercury amalgam, that subsequent electrolytic deposits on the mercury amalgamated surface will be of fine texture and of great tensile strength, the brittleness 100 being greatly reduced if not eliminated.

If desired, the structure may be laminated by the occasional interruption of electrolytic deposit and the application to the surface of the deposited metal of either a film of grease 105 or a film of mercury amalgam.

Where it is necessary or desirable to utilize a non-metallic cathode such as wax or

any electrically non-conductive material removable by a solvent or otherwise, the same being coated with a paint of electrically conductive material, I have found it of great 5 advantage to deposit a relatively thin sheet of copper or other metal on the electrically conductive surface, to treat this surface with mercury and to continue the electrolytic deposit on the amalgamated surface, the second 10 deposit being very fine-grained and of relatively high tensile strength compared with the initial deposit, and the initial deposit being improved in these respects by the combined effects of the mercury, the electrolyte 15 and the current during subsequent electro-deposition.

In my co-pending application, filed here-with, I have described the utilization of grease for purposes of securing improved 20 electro-deposition, and, if desired, to secure a laminated structure. It is obvious that for some purposes a combination of the use of mercury and of grease may be desirable. I have elected to incorporate in the present application those claims of sufficiently broad 25 scope to dominate both inventions. I have used the word "grease" generically to define any substance capable of forming a film of electrically non-conductive material over the 30 surface on which the metal is to be deposited.

After electro-deposition the core of the cathode may be removed by fusion, by burning, by the use of a solvent or any other suitable method.

35 I have utilized the word "galvanoplastic" in its broader sense to include any electrolytic processes in which the entire cathode or any portion thereof is removed subsequent to electro-deposition.

40 It is obvious that the cathode may, if desired, be exterior to the surface thereof on which metal is to be deposited, and that for some purposes my invention may be useful in connection with galvanoplastic processes in 45 which the cathode can be withdrawn without change in the structure thereof.

While I have shown and described one embodiment of my invention and one method of practising the same, it will be understood 50 that major changes may be made, both in the product and the method of producing the

same, without departing from the scope of my invention, which is best defined in the following claims.

55

Claims:

1. The method of forming galvanoplastic products which comprises applying to the surface of a removable, electrically non-conductive mold or core a layer of electrically conductive substance, electrolytically depositing a layer of metal thereon, applying a foreign substance of relatively low tensile strength to the surface of said initial layer of electrolytically deposited metal, continuing electro-deposition to provide a second 60 layer of deposited metal separated from the first by said foreign substance, and subsequently removing the said mold or core.

2. The galvanoplastic process which comprises applying to the surface of a non-conductive mold or core an electrically conductive layer, electrolytically depositing a layer of metal thereon, amalgamating with mercury the surface of the deposited layer, electrolytically depositing a second coating 75 of metal on the amalgamated surface, and subsequently removing the mold or core.

3. The galvanoplastic process which comprises applying to the surface of a non-conductive mold or core an electrically conductive coating, electrolytically depositing a comparatively coarse-grained layer of copper on said conductive layer, amalgamating with mercury the surface of said relatively coarse-grained layer of copper, subsequently 80 electrolytically depositing a second layer of copper, whereby said second layer of copper, partaking of the fine texture of the amalgamated surface, may be of fine grain and of relatively greater strength than the initial 85 layer of copper, and subsequently removing the mold or core.

4. The galvanoplastic process which comprises depositing on the surface of a mold or core successive layers of metal separated by 90 foreign substance of relatively low tensile strength, whereby successive laminations of metallic layers are provided, and subsequently removing the mold or core.

5. In testimony whereof, I have signed my 100 name to this specification.

MATTHEW M. MERRITT.